

## UNITED STATES PATENT OFFICE

2,216,495

## MANUFACTURE OF GOLD ALLOYS

Otto Loebich, Pforzheim, Germany, assignor, by  
mesne assignments, to Chemical Marketing  
Company Inc., New York, N. Y.

No Drawing. Application February 11, 1939, Se-  
rial No. 255,978. In Germany February 2,  
1938

2 Claims. (Cl. 75—165)

My invention relates to the manufacture of gold alloys with a content of gold below 50%.

The hitherto known alloys with a content of gold less than 50% containing besides gold a certain amount of copper, silver and zinc either alone or together, have not proved satisfactory especially with respect to the resistance against tarnishing. The lower the content of gold the more difficult to get the necessary resistance against tarnishing with such alloys since the alloys have also to meet certain requirements in other directions, for instance with respect to the golden color, fusion point, mechanical qualities, workability and so on.

Now it has been found that alloys which contain gold, copper, zinc and palladium and/or platinum in definite quantities have better qualities especially regarding the resistance against tarnishing than the hitherto known alloys with the same or similar contents of gold. Moreover, these new alloys may easily be adapted to the desired requirements with respect to the color of gold or some other qualities.

According to my invention the composition of the gold alloys may be as follows:

25 to 50%, preferably 30 to 45% gold, 15 to 55, preferably 25 to 50% copper, 3 to 30%, preferably 5 to 20% zinc and 1 to 10%, preferably 2 to 8% palladium and/or platinum.

With alloys of the above mentioned composition the platinum metals effect an improvement on the resistance against tarnishing.

An alloy, containing 33.3% of gold, 58% copper and 8.7% zinc and having a red color, for

layer whilst an alloy according to my invention with 33.3% gold, 45% copper, 18.7% zinc and 3% palladium will only be affected to a minor extent.

The fusion points of the above mentioned palladium free alloys and those of the respective alloys which contain palladium are substantially the same. However, the alloys containing palladium show a somewhat increased hardness.

The qualities of the above mentioned alloys containing gold, copper, zinc, palladium and/or platinum may also be affected advantageously by the presence of silver. The quantity of the silver content may amount to 28%, preferably 5 to 25%, calculated on the total alloy.

An alloy with 41.7% gold, 33.3% copper, 10.0% zinc, 8.0% palladium and 7.0% silver with a yellow-reddish color, does not substantially tarnish in sulphuric solutions.

Furthermore, the qualities of the alloys may for instance be influenced by the addition of silver in such a way that the hardness may be increased considerably without deteriorating the resistance against tarnishing. For instance, the addition of silver may increase the hardness of the alloys in soft annealed condition from about 55 to about 70 kgrs./mm.<sup>2</sup> average. Alloys with higher contents of silver, for instance 20%, possess an average hardness of about 115 kgrs./mm.<sup>2</sup> in soft annealed condition. Besides, those alloys may be tempered which may prove advantageous for certain purposes.

The following table shows a summary of silver free and silver containing alloys with statement of hardness and fusion point.

|    | Pd  | Au   | Cu   | Zn   | Ag    | Color               | Hardness               | Average fusion point |
|----|-----|------|------|------|-------|---------------------|------------------------|----------------------|
|    |     |      |      |      |       |                     | Kgrs./mm. <sup>2</sup> | °C.                  |
| 40 | 3.0 | 33.3 | 55   | 8.7  | ----- | Red-----            | 53                     | 930 to 940           |
|    | 3.0 | 33.3 | 45   | 18.7 | ----- | Yellow-----         | 54                     | 920 to 860           |
|    | 5.0 | 37.5 | 39.5 | 10.0 | 8.0   | Reddish-yellow----- | 104                    | 900 to 840           |
|    | 3.0 | 37.5 | 27   | 16.5 | 18.0  | Yellow-----         | 117                    | 810 to 710           |
|    | 3.0 | 33.3 | 37   | 18.7 | 8.0   | Pale-yellow-----    | 67                     | 865 to 800           |
|    | 3.0 | 33.3 | 37.0 | 8.7  | 18.0  | Reddish-yellow----- | 115                    | 860 to 740           |
|    | Pt  | 33.3 | 32.0 | 13.7 | 18.0  | Yellow-----         | 122                    | 840 to 715           |

45 instance, tarnishes in sulphur containing solutions with the formation of a black layer. If the 3% copper have been replaced by 3% palladium, the alloy which now contains 33.3% gold, 55% copper, 8.7% zinc and 3.0% palladium will only be slightly changed by the same sulphuric solution.

A gold alloy of yellow color with 33.3% gold, 48% copper and 18% zinc tarnishes in a sulphuric 55 solution with the formation of a dark brown

In carrying out my invention the alloys may contain other metals to a lesser degree besides the above mentioned components. These are, for instance, aluminium, magnesium, nickel, iron, antimony, tin, cadmium. The alloys may contain up to 5% of those addition metals, calculated on the total alloy. The addition of those metals may influence the qualities of the alloys considerably and make them adapted for the desired requirements. By the addition of iron 50

and nickel the alloys may, for instance, be hardened. By the addition of, for instance, tin, antimony and cadmium the resistance against tarnishing may be improved. Aluminium and magnesium increase the hardness as well as improve the resistance against tarnishing.

5 The following table shows a number of alloys which contain those metals of addition:

| 10 | Pd  | Au   | Cu   | Zn   | Ag |       | Color          | Hardness               | Average fusion point |
|----|-----|------|------|------|----|-------|----------------|------------------------|----------------------|
| 15 | 3.0 | 33.3 | 32.0 | 13.7 | 17 | 1 Mg. | Yellow         | Kgrs./mm. <sup>2</sup> | °C.                  |
|    | 3.0 | 33.3 | 32.0 | 13.7 | 16 | 2 Cd. | do             |                        |                      |
|    | 3.0 | 33.3 | 27.0 | 8.7  | 26 | 2 Al. | do             |                        |                      |
|    | 3.0 | 33.3 | 27.0 | 8.7  | 26 | 2 Fe. | Reddish-yellow |                        |                      |
|    | 3.0 | 33.3 | 45.0 | 8.7  | 8  | 2 Al. | do             |                        |                      |
|    | 3.0 | 33.3 | 45.0 | 8.7  | 8  | 2 Ni  | Red            |                        |                      |

If platinum metals such as iridium and/or 20 rhodium are added to the alloys in quantities of about 0.001 to 0.1% considerable crystalline refinements may be obtained. It has been found, for instance, that alloys of the above mentioned 25 composition to which iridium has been added in quantities of, for instance, 0.1/000 after rolling and annealing had a substantially fine-grained structure. As some of the alloys made according to my invention as a consequence to the 30 supplemental use of grain refining additions has

special advantages, as the perhaps occurring difficulties decrease by enhancing the fineness of the grain of the alloy.

It has proved advantageous to add the grain refining additions in the form of preliminary alloys with base metals, such as for instance tin, cadmium and the like. In this case preferably such base metals are used for the manufacture

10.

15.

20.

30.

of the preliminary alloys which form a pre-destined part of the resulting alloy.

What I claim is:

1. Gold alloy consisting of 25 to 50% gold, 15 to 55% copper, 3 to 30% zinc, 1 to 10% of a metal selected from the group consisting of palladium and platinum and an addition up to 25% silver. 25

2. Gold alloy consisting of 30 to 45% gold, 25 to 50% copper, 5 to 20% zinc, 2 to 8% of a metal selected from the group consisting of palladium and platinum, about 25% silver.

OTTO LOEBICH. 30